



US009221579B2

(12) **United States Patent**  
**Thorstensen-Woll**

(10) **Patent No.:** **US 9,221,579 B2**  
(45) **Date of Patent:** **\*Dec. 29, 2015**

(54) **INNER SEAL WITH A SUB TAB LAYER**(71) Applicant: **Selig Sealing Products, Inc.**, Forrest, IL (US)(72) Inventor: **Robert William Thorstensen-Woll**, Barrie (CA)(73) Assignee: **SELIG SEALING PRODUCTS, INC.**, Forrest, IL (US)

(\* ) Notice: Subject to any disclaimer, the term of this patent is extended or adjusted under 35 U.S.C. 154(b) by 0 days.

This patent is subject to a terminal disclaimer.

(21) Appl. No.: **14/681,649**(22) Filed: **Apr. 8, 2015**(65) **Prior Publication Data**

US 2015/0225116 A1 Aug. 13, 2015

**Related U.S. Application Data**

(63) Continuation of application No. 14/208,122, filed on Mar. 13, 2014.

(60) Provisional application No. 61/791,788, filed on Mar. 15, 2013.

(51) **Int. Cl.**

**B65D 17/00** (2006.01)  
**B65D 17/50** (2006.01)  
**B65D 51/20** (2006.01)  
**B65D 43/02** (2006.01)  
**B65D 51/00** (2006.01)

(52) **U.S. Cl.**

CPC ..... **B65D 17/163** (2013.01); **B65D 17/50** (2013.01); **B65D 43/02** (2013.01); **B65D 51/005** (2013.01); **B65D 51/20** (2013.01); **B65D 2251/0015** (2013.01); **B65D 2251/0018** (2013.01); **B65D 2251/0071** (2013.01); **B65D**

2251/0093 (2013.01); **B65D 2517/0013** (2013.01); **B65D 2517/0082** (2013.01); **B65D 2577/2058** (2013.01); **Y10T 428/12486** (2015.01)

(58) **Field of Classification Search**None  
See application file for complete search history.(56) **References Cited**

## U.S. PATENT DOCUMENTS

2,768,762 A \* 10/1956 Guinet ..... 215/320  
3,235,165 A 2/1966 Jackson

(Continued)

## FOREIGN PATENT DOCUMENTS

AT 501393 A1 8/2006  
AT 11738 U1 4/2011

(Continued)

## OTHER PUBLICATIONS

Search Report in European Application No. 14160375.3, dated Jun. 23, 2014, 4 pages.

(Continued)

*Primary Examiner* — David Sample*Assistant Examiner* — Donald M Flores, Jr.(74) *Attorney, Agent, or Firm* — Fitch, Even, Tabin & Flannery LLP(57) **ABSTRACT**

A pull-tab sealing member for a container containing an upper laminate forming a pull-tab bonded to a lower laminate capable of being heat sealed to a container's mouth or opening. The upper laminate defines the pull tab wholly within a perimeter or circumference of the seal. The sealing member further includes a sub tab layer or member under the gripping tab for concentric structural support.

**24 Claims, 6 Drawing Sheets**

| References Cited         |         |                 |                    |
|--------------------------|---------|-----------------|--------------------|
| U.S. PATENT DOCUMENTS    |         |                 |                    |
| 3,292,828 A              | 12/1966 | Stuart          | 7,740,927 B2       |
| 3,302,818 A              | 2/1967  | Balocca et al.  | 7,789,262 B2       |
| 3,460,310 A              | 8/1969  | Adcock et al.   | 7,798,359 B1       |
| 3,990,603 A              | 11/1976 | Brochman        | 7,819,266 B2       |
| 4,133,796 A              | 1/1979  | Bullman         | 7,838,109 B2       |
| 4,206,165 A              | 6/1980  | Dukess          | 7,850,033 B2       |
| 4,582,735 A              | 4/1986  | Smith           | 8,057,896 B2       |
| 4,588,099 A              | 5/1986  | Diez            | 8,329,288 B2       |
| 4,596,338 A              | 6/1986  | Yousif          | 8,348,082 B2       |
| 4,636,273 A              | 1/1987  | Wolfersperger   | 2002/0068140 A1    |
| 4,666,052 A              | 5/1987  | Ou-Yang         | 2003/0168423 A1    |
| 4,735,335 A              | 4/1988  | Torterotot      | 2004/0043238 A1    |
| 4,741,791 A              | 5/1988  | Howard          | 2004/0109963 A1    |
| 4,770,325 A              | 9/1988  | Gordon          | 2005/0048307 A1    |
| 4,801,647 A              | 1/1989  | Wolfe, Jr.      | 2005/0208242 A1 *  |
| 4,811,856 A              | 3/1989  | Fischman        | 2006/0000545 A1    |
| 4,837,061 A              | 6/1989  | Smits           | 2006/0003120 A1    |
| 4,960,216 A              | 10/1990 | Giles           | 2006/0003122 A1    |
| 4,961,986 A              | 10/1990 | Galda           | 2006/0151415 A1    |
| 5,004,111 A              | 4/1991  | McCarthy        | 2006/0278665 A1    |
| 5,015,318 A              | 5/1991  | Smits           | 2007/0003725 A1    |
| 5,055,150 A              | 10/1991 | Rosenfeld       | 2007/0065609 A1    |
| 5,057,365 A              | 10/1991 | Finkelstein     | 2007/0267304 A1    |
| 5,071,710 A              | 12/1991 | Smits           | 2007/0298273 A1    |
| 5,098,495 A              | 3/1992  | Smits           | 2008/0026171 A1    |
| RE33,893 E               | 4/1992  | Elias           | 2008/0073308 A1    |
| 5,125,529 A              | 6/1992  | Torterotot      | 2008/0103262 A1    |
| 5,149,386 A              | 9/1992  | Smits           | 2008/01078671 A1   |
| 5,178,967 A              | 1/1993  | Rosenfeld       | 2009/0078671 A1    |
| 5,197,618 A              | 3/1993  | Goth            | 2009/0208729 A1    |
| 5,265,745 A              | 11/1993 | Pereyra         | 2009/0304964 A1    |
| 5,433,992 A              | 7/1995  | Galda           | 2010/0009162 A1    |
| 5,513,781 A              | 5/1996  | Ullrich         | 2010/0030180 A1    |
| 5,514,442 A              | 5/1996  | Galada et al.   | 2010/0047552 A1    |
| 5,598,940 A              | 2/1997  | Finkelstein     | 2010/0059942 A1    |
| 5,601,200 A              | 2/1997  | Finkelstein     | 2010/0116410 A1    |
| 5,615,789 A              | 4/1997  | Finkelstein     | 2010/0155288 A1    |
| 5,669,521 A              | 9/1997  | Wiening         | 2010/0170820 A1    |
| 5,702,015 A              | 12/1997 | Giles           | 2010/0193463 A1    |
| 5,860,544 A              | 1/1999  | Brucker         | 2010/0213193 A1    |
| 5,871,112 A              | 2/1999  | Giles           | 2010/0221483 A1    |
| 5,915,577 A              | 6/1999  | Levine          | 2010/0290663 A1    |
| 5,975,304 A              | 11/1999 | Cain            | 2010/0314278 A1    |
| 6,082,566 A              | 7/2000  | Yousif          | 2011/0000917 A1    |
| 6,096,358 A              | 8/2000  | Murdick         | 2011/0005961 A1    |
| 6,131,754 A              | 10/2000 | Smelko          | 2011/0089177 A1    |
| 6,139,931 A              | 10/2000 | Finkelstein     | 2011/0091715 A1    |
| 6,158,632 A              | 12/2000 | Ekkert          | 2011/0100949 A1    |
| 6,194,042 B1             | 2/2001  | Finkelstein     | 2011/0100989 A1    |
| 6,312,776 B1             | 11/2001 | Finkelstein     | 2011/0138742 A1    |
| 6,378,715 B1             | 4/2002  | Finkelstein     | 2011/0147353 A1    |
| 6,458,302 B1             | 10/2002 | Shiftlet        | 2012/0000910 A1    |
| 6,548,302 B1             | 4/2003  | Mao             | 2012/0043330 A1    |
| 6,602,309 B2             | 8/2003  | Vizulis         | 2012/0067896 A1    |
| 6,627,273 B2             | 9/2003  | Wolf            | 2012/0103988 A1    |
| 6,699,566 B2             | 3/2004  | Zeiter          | 2012/0111758 A1 *  |
| 6,705,467 B1             | 3/2004  | Kancsar         | 2012/0241449 A1    |
| 6,722,272 B2             | 4/2004  | Jud             | 2013/0020324 A1    |
| 6,767,425 B2             | 7/2004  | Meier           | 2014/0061196 A1    |
| 6,790,508 B2             | 9/2004  | Razeti          | 2014/0186589 A1    |
| 6,866,926 B1             | 3/2005  | Smelko          |                    |
| 6,902,075 B2             | 6/2005  | OBrien          |                    |
| 6,916,516 B1             | 7/2005  | Gerber          |                    |
| 6,955,736 B2             | 10/2005 | Rosenberger     | BR 8200231 U       |
| 6,974,045 B1             | 12/2005 | Trombach        | BR 0300992 A       |
| 7,128,210 B2             | 10/2006 | Razeti          | CA 2015992 A1      |
| 7,182,475 B2             | 2/2007  | Kramer          | DE 102006030118 B3 |
| 7,217,454 B2             | 5/2007  | Smelko          | DE 10204281 A1     |
| RE39,790 E               | 8/2007  | Fuchs           | DE 102007022935 B4 |
| 7,316,760 B2             | 1/2008  | Nageli          | DE 202009000245 U1 |
| 7,448,153 B2             | 11/2008 | Maliner         | EP 0668221 A1      |
| 7,531,228 B2             | 5/2009  | Perre           | EP 0826598 A2      |
| 7,648,764 B2             | 1/2010  | Yousif          | EP 0826599 A2      |
| 7,713,605 B2             | 5/2010  | Yousif          | EP 0717710 B1      |
| 7,740,730 B2             | 6/2010  | Schedl          | EP 0915026 A1      |
| FOREIGN PATENT DOCUMENTS |         |                 |                    |
|                          | BR      | 8200231 U       | 9/2003             |
|                          | BR      | 0300992 A       | 11/2004            |
|                          | CA      | 2015992 A1      | 1/1991             |
|                          | DE      | 102006030118 B3 | 5/2007             |
|                          | DE      | 10204281 A1     | 8/2007             |
|                          | DE      | 102007022935 B4 | 4/2009             |
|                          | DE      | 202009000245 U1 | 4/2009             |
|                          | EP      | 0668221 A1      | 8/1995             |
|                          | EP      | 0826598 A2      | 3/1998             |
|                          | EP      | 0826599 A2      | 3/1998             |
|                          | EP      | 0717710 B1      | 4/1999             |
|                          | EP      | 0915026 A1      | 5/1999             |

| (56)                     | <b>References Cited</b> |               | MX                                                                                  | 2010001867 A  | 4/2010        |        |
|--------------------------|-------------------------|---------------|-------------------------------------------------------------------------------------|---------------|---------------|--------|
|                          | WO                      | 9905041 A1    | 2/1999                                                                              |               |               |        |
|                          | WO                      | 0066450       | 11/2000                                                                             |               |               |        |
|                          | WO                      | 2006018556 A1 | 2/2006                                                                              |               |               |        |
|                          | WO                      | 2006021291 A1 | 3/2006                                                                              |               |               |        |
| FOREIGN PATENT DOCUMENTS |                         | WO            | 2006073777 A1                                                                       | 7/2006        |               |        |
| EP                       | 0706473 B1              | 8/1999        | WO                                                                                  | 2006108853 A1 | 10/2006       |        |
| EP                       | 1075921 A2 *            | 2/2001        | ..... B29C 47/06                                                                    | WO            | 2008027029 A2 | 3/2008 |
| EP                       | 0803445 B1              | 11/2003       | WO                                                                                  | 2008027036 A1 | 3/2008        |        |
| EP                       | 1462381 A1              | 9/2004        | WO                                                                                  | 2008039350 A2 | 4/2008        |        |
| EP                       | 1199253 B1              | 3/2005        | WO                                                                                  | 2008125784 A1 | 10/2008       |        |
| EP                       | 1577226 A1              | 9/2005        | WO                                                                                  | 2008125785 A1 | 10/2008       |        |
| EP                       | 1814744 A1              | 8/2007        | WO                                                                                  | 2008148176 A1 | 12/2008       |        |
| EP                       | 1834893 A1              | 9/2007        | WO                                                                                  | 2009092066 A2 | 7/2009        |        |
| EP                       | 1837288 A1              | 9/2007        | WO                                                                                  | 2010115811 A1 | 10/2010       |        |
| EP                       | 1839898 A1              | 10/2007       | WO                                                                                  | 2011039067 A1 | 4/2011        |        |
| EP                       | 1839899 A1              | 10/2007       | WO                                                                                  | 2012079971 A1 | 6/2012        |        |
| EP                       | 1857275 A1              | 11/2007       | WO                                                                                  | 2012113530 A1 | 8/2012        |        |
| EP                       | 1873078 A1              | 1/2008        | WO                                                                                  | 2012152622 A1 | 11/2012       |        |
| EP                       | 1445209 B1              | 5/2008        | WO                                                                                  | 2012172029 A1 | 12/2012       |        |
| EP                       | 1918094 A1              | 5/2008        |                                                                                     |               |               |        |
| EP                       | 1968020 A1              | 9/2008        |                                                                                     |               |               |        |
| EP                       | 1992476 A1              | 11/2008       |                                                                                     |               |               |        |
| EP                       | 2230190 A1              | 9/2010        |                                                                                     |               |               |        |
| EP                       | 2292524 A1              | 3/2011        |                                                                                     |               |               |        |
| FR                       | 2916157 A1              | 11/2008       | Search Report in European Application No. 14160367.0, dated Jun. 23, 2014, 4 pages. |               |               |        |
| FR                       | 2943322 A1              | 9/2010        | Search Report in European Application No. 14160374.6, dated Jun. 16, 2014, 5 pages. |               |               |        |
| KR                       | 100711073 B1            | 4/2007        |                                                                                     |               |               |        |
| KR                       | 100840926 B1            | 6/2008        |                                                                                     |               |               |        |
| KR                       | 100886955 B1            | 3/2009        |                                                                                     |               |               |        |
| MX                       | 05002905 A              | 2/2006        |                                                                                     |               |               |        |

\* cited by examiner

FIG. 1



**FIG. 2**



**FIG. 3****FIG. 4**

**FIG. 6****FIG. 7**

FIG. 8



FIG. 9



**FIG. 10****FIG. 11**

## 1

## INNER SEAL WITH A SUB TAB LAYER

## CROSS-REFERENCE TO RELATED APPLICATIONS

This application is a continuation of prior application Ser. No. 14/208,122, filed Mar. 13, 2014, which claims benefit of U.S. Provisional Application No. 61/791,788, filed Mar. 15, 2013, both of which are hereby incorporated herein by reference in their entirety.

## FIELD

The disclosure relates to a pull-tab sealing member for closing the mouth of a container, and more particularly, to a pull-tab sealing member having a tab formed with a sub tab layer underneath to provide concentric stability between peripheral portions of the sealing member and central portions of the sealing member during heat sealing to a container rim.

## BACKGROUND

It is often desirable to seal the opening of a container using a removable or peelable seal, sealing member, or inner seal. Often a cap or other closure is then screwed or placed over the container opening capturing the sealing member therein. In use, a consumer typically removes the cap or other closure to gain access to the sealing member and then removes or otherwise peels the seal from the container in order to dispense or gain access to its contents.

Initial attempts at sealing a container opening utilized an induction- or conduction-type inner seal covering the container's opening where the seal generally conformed to the shape of the opening such that a circular container opening was sealed with a round disk approximately the same size as the opening. These prior seals commonly had a lower heat activated sealing layer to secure a periphery of the seal to a rim or other upper surface surrounding the container's opening. Upon exposing the seal to heat, the lower layer bonded to the container's rim. In many cases, these seals included a foil layer capable of forming induction heat to activate the lower heat seal layer. These prior seals tended to provide good sealing, but were often difficult for a consumer to remove because there was nothing for the consumer to grab onto in order to remove the seal. Often, the consumer needed to pick at the seal's edge with a fingernail because there was little or no seal material to grasp.

Other types of seals for containers include a side tab or other flange that extended outwardly from a peripheral edge of the seal. These side tabs are generally not secured to the container rim and provide a grasping surface for a consumer to hold and peel off the seal. These side tabs, however, extend over the side of the container rim and often protrude into a threaded portion of the closure. If the side tab is too large, this configuration may negatively affect the ability of the seal to form a good heat seal. The side tabs (and often the seal itself) can be deformed or wrinkled when the closure or other cap is placed on the container due to contact between the closure (and threads thereof) and tabbed part of the seal. To minimize these concerns, the side tabs are often very small; thus, providing little surface area or material for a consumer to grasp in order to remove the seal.

Yet other types of seals include a sealing member having a tab defined on the top of the seal. One approach of these prior seals includes a partial layer of coated pressure sensitive adhesive to secure the tab to a layer of metal foil. The tab was

## 2

formed by a full layer extending across the entire surface of the sealing member, but the full layer was only bonded to half of the seal to form the tab. This type of top-tabbed seal offered the advantage of a larger tab, which provided more grasping area for the consumer to hold and peel off the seal, but required a full additional layer of material in order to form the tab. In other approaches, the seal may include a tab formed from the additional full layer of film combined with an additional full layer of adhesive utilizing a part paper or part polymer layer, called a tab stock, to form the tab. This part layer is inserted between the additional full layer of adhesive and lower seal portions to prevent the tab from sticking to the layers below, which formed the tab. In all the prior types of top-tabbed-like seals, the gripping tab was formed by a full layer of material (or a full layer of material and a full layer of adhesive) that extended across the entire surface of the seal.

As mentioned above, a cap or other closure is typically screwed or otherwise secured to a finish or neck of a container. This captures the sealing member between the top of the cap and container rim. In many instances, the cap has an annular bead or downwardly protruding ring (sometimes called a bead line) on the underside of its top inner surface. This annular bead is sized and positioned to generally correspond with an upper land area of the container rim when the cap is secured to the container. This annular bead helps provide pressure to secure the sealing member to the rim land area. However, many of the prior sealing members included a foam layer to provide insulation from heat generated during the heat sealing process. In some cases, there can be problems with the foam layer interacting with the cap annular bead during the cap sealing process. Heat from the cap sealing process combined with the focused downward pressure from the annular bead on the foam layer in the sealing member can damage or result in deterioration of the foam layer in the areas above the container rim. In extreme cases, the foam may melt or air cells in the foam may collapse. This shortcoming is more prevalent when the cap sealing process is over sealed (that is, when too much heat is applied or heat is applied for too long during the cap sealing process).

This melting and/or cell collapse may result in exposure of the metal foil or other polymer layers below the foam at the peripheral areas of the sealing member. In some cases, when the consumer lifts up the tab to remove the sealing member, the consumer is presented with an unsightly seal having an uneven foam layer under the tab with intact center portions of foam and melted or damaged edge portions of the foam. In extreme cases, the outer peripheral portions of the foam may melt completely, which exposes the metal foil or other layers under the tab.

## BRIEF DESCRIPTION OF THE DRAWINGS

FIG. 1 is a perspective view of an exemplary tabbed sealing member;

FIG. 2 is a cross-sectional view of another exemplary sealing member;

FIG. 3 is an exploded perspective view of another exemplary sealing member;

FIG. 4 is a cross-sectional view of another exemplary sealing member;

FIG. 5 is an exploded perspective view of another exemplary sealing member;

FIG. 6 is a cross-sectional view of another exemplary sealing member;

FIG. 7 is a cross-sectional view of another exemplary sealing member temporarily bonded to a liner via a wax or other release layer;

FIGS. 8 and 9 are top plan views of exemplary tabbed sealing members;

FIG. 10 is a cross-sectional view of another exemplary tabbed sealing member; and

FIG. 11 is a cross-sectional view of another exemplary tabbed sealing member.

#### DETAILED DESCRIPTION

When confronted with a heat management problem during a cap sealing process, such as the one set forth in the background, the conventional approach would be to add more insulation. In the case of tabbed sealing members with a foam layer, additional insulation may be obtained by adding further foamed polymers or by increasing the thickness of any existing foamed polymer layers. It is well understood that foaming of a polymer layer decreases its thermal conductivity and, thus, increases the ability of the foamed polymer to provide insulation and hinder the transfer of heat. Thicker foams would also logically compensate for the added pressure due to the cap's annular bead. Thus, the logical approach to solve the deteriorating foam issues of prior sealing members would have been to include a thicker foam layer or include additional foam layers to provide more insulation to hinder the flow of heat and/or to better absorb the downward pressure from the cap's annular bead.

The tabbed sealing members of the present application, however, take the unconventional approach of including one or more non-foamed, polymer layers between a tab and a foamed polymer layer in a seal laminate to provide a more robust tabbed sealing member. The sealing members of the present application are unexpectedly better able to withstand additional or excessive heating during the cap sealing process when combined with a cap or closure including the annular bead on its inner surface. The approach of the present application is unconventional because the non-foamed, polymer layer(s) have a higher thermal conductivity and are more rigid (as compared to foam) and would be expected to conduct more heat and not absorb the downward pressure of the cap as well as foam during the cap sealing process.

It was unexpectedly discovered that including one or more of these non-foamed, polymer layers between the tab and the foam actually helped reduce foam damage due to melting and cell collapse at the outer peripheral edge when the tabbed sealing members are exposed to excessive heating and the cap's annular bead during a cap sealing process. In some approaches, the non-foam, polymer layer(s) are positioned in the laminate between the tab and foam layers to be at least co-extensive with a peripheral edge of the tab and to extend inwardly along with the tab only part way across the seal. In other approaches, the non-foam, polymer layer(s) may also extend over the entire seal structure. In this manner, the non-foam, polymer layer(s) provides improved concentric stability to the sealing member and to the foamed polymer layer under the tab during cap sealing process. Concentric stability is the ability of the tabbed sealing member to generally maintain the integrity and cell structure of the foamed polymer layer at its peripheral edge above the container rim land area generally consistent with the integrity and cell structure of the foam layer at radially inner portions away from the edge. This concentric stability is achieved via the unconventional approach of using a thermally conductive and more rigid non-foam polymer rather than the conventional approach of using additional or thicker foamed insulation layers to address issues with the flow of heat and added pressure of the cap's annular bead during cap sealing.

In a first aspect, this disclosure provides a concentrically stable tabbed sealing member with a foam layer therein for sealing to a rim surrounding a container opening. The concentrically stable tabbed sealing member includes a multi-layer laminate with an upper laminate portion partially bonded to a lower laminate portion forming a gripping tab defined wholly within a perimeter of the sealing member. The gripping tab is arranged and configured for removing the sealing member from a container opening. The lower laminate portion below the gripping tab (such as when viewed through a cross-section extending through the tab) includes at least a seal layer for bonding to the container rim, a metal layer for heating the seal layer, and a polymer foam layer above the metal layer. Other layers may be included as needed.

To provide concentric structural support, the tabbed sealing members, in one approach (when viewed, for instance, through a cross-section extending through the tab), include one or more non-foam, polymer sub-tab layers between the polymer foam layer and the gripping tab. The non-foam, polymer sub-tab layer may be bonded to the upper surface of the lower laminate which may be a foam layer. In some approaches, the one or more non-foam, polymer sub-tab layers may be coextensive with at least the gripping tab at a periphery thereof. For instance, the one or more non-foam, polymer sub-tab layers may be partial layers coextensive with the tab or, as discussed more below, coextensive with a so-called tab stock layer. In other approaches, the one or more non-foam, polymer sub-tab layers may also extend over the entire sealing member between the upper laminate portion and polymer foam layer of the lower laminate portion. Even though the sub-tab layer is a non-foam polymer and tends to conduct more heat than a foamed polymer, it provides concentric structural support to the polymer foam layer at its periphery thereof relative to portions of the polymer foam layer radially inward from the periphery when exposed to heating and the cap's annular bead during a cap sealing process.

In another approach, this disclosure also includes a container and cap assembly that includes the concentrically stable tabbed sealing member with foam mentioned above. The container includes a rim surrounding an opening thereof, and the cap closes the opening of the container. The cap includes a downwardly extending annular bead on a top inner surface thereof. The annular bead is arranged and configured to generally align with a land area of the container rim when the cap is received on a neck or other finish of the container.

In yet another approach, a pull-tab sealing member for a container is described herein containing an upper laminate forming a pull-tab bonded to a lower laminate capable of being heat sealed to a container's mouth or opening. The upper laminate defines a pull tab wholly within a perimeter or circumference of the seal. The sealing member includes a sub tab polymer layer underneath the tab and bonded to the lower laminate, but not bonded to the tab itself. This sub tab layer adds structural support to stabilize the sealing member and tab to aid in minimizing folding, wrinkles, creases, and the like. The sub tab polymer layer can be coextensive with the tab, extend slightly beyond the tab, but not extend the full width of the sealing member, or the sub-tab polymer layer may extend the full surface area of the sealing member. For instance, the sub tab polymer layer may be coextensive with a tab stock, be coextensive with the full upper laminate, or, may be other sizes as needed for a particular application. This sub tab polymer layer can, in some approaches, be particularly advantageous in seals with relatively thin lower laminates (such as about 3 mils or less), but can be used in a wide

variety of seals needing structural support with a tab. The sub tab layer may aid in providing concentric stability of the sealing member.

In other aspects of this disclosure, the upper laminate of the seal does not extend the full width of the sealing member in order to define the gripping tab. To this end, the pull-tab sealing members herein may also combine the advantages of a tabbed sealing member with a large gripping tab defined completely within the perimeter of the seal, but achieve such functionality with less material (in view of the part layers of the upper laminate) and permit such a tab structure to be formed on many different types of pre-formed lower laminates. This partial upper laminate can be combined with the sub tab layer described above and/or additional upper layers (such as a full paper layer) as needed for particular applications. The partial upper laminate structure is advantageous, in some approaches, for use with a seal configured for large or wide mouth containers, such as containers with an opening from about 30 to about 100 mm (in other approaches, about 60 to about 100 mm). These seals may also be used with 38 mm or 83 mm container openings, or can be used with any sized container.

In yet another aspect of this disclosure, the tab may be formed by a full layer or partial layer of material combined with a partial width composite adhesive structure that includes a polyester core with upper and lower adhesives on opposite sides thereof. This partial composite adhesive structure bonds the upper laminate to the lower laminate to form the gripping tab. The partial composite adhesive structure may also be combined with the above mentioned sub tab layers. In this approach, the sub tab is adhered to the lower laminate and not adhered to the upper laminate to enhance structural support.

In further aspects of this disclosure, the sealing members herein may include a pull or grip tab defined in the upper laminate portion wholly within a perimeter or circumference of the sealing member wherein an upper surface of the sealing member is partially defined by the upper laminate portion and partially defined by the lower laminate portion. In one approach of this aspect, the top surface of the sealing member is provided by a minor portion of the upper laminate and a major portion of the lower laminate. In other approaches of this aspect, the lower laminate is partially exposed at a top surface of the seal with about 50 percent to about 75 percent (or more) of the lower laminate exposed at the top surface of the entire seal. The seals of this aspect allow consumers to remove the sealing member using the tab (as in a conventional pull-tab seal) and/or puncture the sealing member by piercing the exposed lower laminate portion to provide push/pull functionality depending on the preference of the consumer. Prior tabbed seals having a top-defined gripping tab via a full width film layer generally did not allow the functionality of easy piercing because the additional full layers used to form the tab rendered the seal too difficult to pierce.

In such aspects, the seals of the present disclosure defining a tab wholly within a perimeter or circumference of the seal (but formed by a partial layer) also provide an improved ability for the tabbed sealing member to function in a two-piece seal and liner combination. In a two-piece seal and liner combination, the tabbed sealing member is temporarily adhered across its top surface to a liner. After container opening and removal of a cap or closure, the sealing member stays adhered to the container mouth and the liner separates and remains in the container's cap.

In some prior versions of two-piece seal and liner assemblies, the bottom layer of the sealing member is a heat seal layer that is activated by heating, such as by induction or

conduction heating, in order to adhere or bond an outer periphery of the sealing member to a rim surrounding the mouth of a container. In the two-piece seal and liner combination, an upper surface of the sealing member is temporarily adhered to a lower surface of the liner by a release layer, which is often a heat-activated release layer, such as an intervening wax layer. During heating to bond the sealing member to the container, heat not only activates the lower heat seal layer, but also travels upwardly through the seal to melt the intervening wax across the entire surface of the sealing member to separate the liner from the sealing member. Often, the melted wax is absorbed by the liner in order to permit easy liner separation from the sealing member. As can be appreciated, for this sealing member and liner combination to function properly, the intervening wax layer needs to be melted across the entire surface of the sealing member. If the wax is not melted evenly all the way across the sealing member upper surface, the liner may not properly separate from the lower seal portion.

As the prior tabbed seals required additional full layers of material (film and adhesive) to form the tab, these additional layers would tend to negatively affect heat transfer upwardly through the seal. This shortcoming of less upward heat transfer limits the ability of top-tabbed-type seals to be used in the two-component liner and seal assembly because the required additional full layers of material (film and adhesive) to form the tab often led to issues with the proper melting the wax for liner separation.

These shortcomings of prior tabbed seals in the context of a two-piece liner and seal combinations tended to be even more pronounced in view of further shortcomings of some induction heating equipment. In an induction seal, a metal foil is often included in the seal to generate heat for activation of the heat seal. This heat is generated due to the induction apparatus forming eddy currents in the foil layer. The induction heat from the foil melts the lower heat seal layer for bonding to the container rim. In a common two-piece assembly, the induction heating generated by the foil layer is also used to melt the intervening wax layer (as mentioned above); however, the induction heating generated by the foil layer at the center of the seal is often lower than the induction heating generated by the foil at the periphery of the seal laminate. The center of the laminate is farthest away from the induction coil in the induction heating apparatus and the eddy currents in the foil are weakest at the center of the disk, which can form a cold spot in the center of the seal. This shortcoming tends to be further exaggerated in wide seals (such as those about 60 mm in diameter or larger or seals about 60 to about 100 mm across) because the center is much farther from the induction coil. Normally, such variation in induction heating between the edges of the seal laminate and the center is generally not an issue because heat is needed most at the seal's periphery for bonding to the container rim at the periphery of the seal laminates. In prior two-piece seals without top-oriented tabs, there was less material to hinder the upwardly directed flow of heat. However, when attempting to use the top-type-tabbed seals in a two-piece liner and seal combination, the extra full layers forming the tab often created problems when attempting to use induction heat to melt the intervening wax layer, especially in the center of the seal where the induction heating was the lowest.

In further approaches of this disclosure, the tab is formed wholly within a perimeter of the sealing member, but the upper laminate and layers forming that tab are spaced from central portions and regions of the sealing member. In some approaches, the layers defining the tab in the upper laminate are provided by a circular segment that is less than a semi-

circle within the sealing member's upper surface. As discussed more below, in some approaches, the upper laminate circular segment forming the tab is defined by a chord (that does not extend through the center of the sealing member) and the perimeter of the sealing member along its circumference between opposing endpoints of the chord. In this manner, the lower laminate is exposed at the center and center portions of the seal so that the center portions are free of the layers forming the tab (and upper laminate). This is advantageous in a two-piece assembly because it permits greater upwardly directed heat flow in the center portions of the seal to melt the intervening wax layer more easily than the prior tabbed seals.

Turning to more of the specifics, FIGS. 1 and 2 generally show a tabbed seal 10 having an upper laminate 12 and a lower laminate 14. The upper laminate 12 defines a grip tab 16 wholly within a circumference or perimeter 18 of the seal 10. By one approach, the upper laminate 12 is formed by one or more layers of adhesive and/or film where all layers forming the upper laminate 12 and the defined grip tab 16 extend only partway across an upper or major surface of the lower laminate 14. In this form, the upper laminate 12 forms a circular segment defined by edges of the upper laminate 12 where one edge 20 is a chord of the seal 10 and another edge 22 is a segment extending along the perimeter or circumference 18 between opposing chord endpoints 24 and 26. As shown in this exemplary approach, the upper laminate, circular segment 12 is spaced a distance 28 from the center C of the seal 10. In this manner, the center portions or regions of the seal 10 are free of the upper laminate 12. In such approach, an upper surface 32 of the lower laminate 14 is exposed at a top surface of the seal, and in some cases, is exposed for at least about 50 percent and, in some cases, greater than half of the sealing member 10. In other approaches, the upper surface 32 of the lower laminate 14 is exposed for about 50 to about 75 percent of the sealing member's upper total surface area. The upper laminate 12 defining the gripping tab may also extend the full width and full surface area of the seal 10 as needed for particular applications.

For simplicity, this disclosure generally may refer to a container or bottle, but the sealing members herein may be applied to any type of container, bottle, package or other apparatus having a rim or mouth surrounding an access opening to an internal cavity. In this disclosure, reference to upper and lower surfaces and layers of the components of the sealing member refers to an orientation of the components as generally depicted in figures and when the sealing member is in use with a container in an upright position and having an opening at the top of the container. Different approaches to the sealing member will first be generally described, and then more specifics of the various constructions and materials will be explained thereafter. It will be appreciated that the sealing members described herein, in some cases, function in both a one-piece or two-piece sealing member configuration. A one-piece sealing member generally includes just the sealing member bonded to a container rim. A cap or closure may be also used therewith. A two-piece sealing member includes the sealing member temporarily bonded to a liner. In this construction, the sealing member is bonded to a container's rim, and the liner is configured to separate from the sealing member during heating to be retained in a cap or other closure used on the container. In a two-piece construction, a wax layer, for example, may be used to temporarily bond the sealing member to a liner. Other types of releasable layers may also be used to provide a temporary bond between the seal and liner, but the releasable layers are generally heat activated.

In this first approach, the circular segment forming the upper laminate 12 includes the tab portion 16, which is free to

pivot upwardly at a pivot line 34 because the tab 16 is not adhered to the lower laminate 14. The circular segment forming the upper laminate 12 also includes an adhered portion 30 that is directly bonded to the lower laminate 14 or any intervening layers between the upper and lower laminates. The adhered portion 30 extends between the pivot line 34 and segment chord 20. In some approaches (turning to FIG. 9 for a moment), the adhered portion 30 of the upper laminate circular segment 12 may have a length or height H1 that is about 30 to about 75 percent of the total length or height H of the upper laminate circular segment laminate 12 and, in other approaches, about 40 to about 60 percent of the laminate 12, and in yet other approaches, about 30 to about 40 percent of the laminate 12 and still provides a strong bond so that the tab 16 may be used to pull the sealing member 10 from a container rim in one piece. The tab 16 of the upper laminate circular segment 12 has a height or length H2 being the remainder of the upper laminate circular segment 12, and in some cases the tab 16 is the majority of the segment 12. In another approach, the circular segment 12 may define a ratio of tab 16 to adhered portion 30 of about 1:1 to about 2.5:1 and, in other approaches, may be about 1.1 to about 2.1:1.

The lower laminate 14 is not particularly limited and can be any single or multiple layer film structure, sheet, or laminate as needed for a particular application. For instance, lower laminate 14 may be from about 1 mil to about 20 mils thick, and in some approaches, about 7 to about 10 mils thick and include a lower heat seal layer for bonding to a container rim, a metal layer for heating the heat seal layer, and a polymer foam layer above the metal layer. In some approaches, however, particular laminate structures of the lower laminate 14 are more advantageous for certain applications. FIGS. 3-7 provide examples of various laminates suitable the lower laminate 14. In yet other approaches, the sub-tab layer is provided between the tab or upper laminate including the tab and the lower laminate and the foam in the lower laminate.

In FIGS. 3 and 4, another example of a seal 10 is provided. In this approach, the lower laminate 14 may include, from bottom to top, a lower sealant or heat seal layer 100, a polymer film support layer 102 above and over the seal layer 100, a membrane or an induction heatable layer 104 above the support layer. On top of the membrane layer 104 may be an insulation layer or heat redistribution 106 and an optional top non-foam polymer support layer 108. Each of these layers will be described more below.

The lower sealant or heat seal layer 100 may be composed of any material suitable for bonding to the rim of a container, such as but not limited to induction, conduction, or direct bonding methods. Suitable adhesives, hot melt adhesives, or sealants for the heat sealable layer 100 include, but are not limited to, polyesters, polyolefins, ethylene vinyl acetate, ethylene-acrylic acid copolymers, surlyn, and other suitable materials. By one approach, the heat sealable layer may be a single layer or a multi-layer structure of such materials about 0.2 to about 3 mils thick. By some approaches, the heat seal layer is selected to have a composition similar to and/or include the same polymer type as the composition of the container. For instance, if the container includes polyethylene, then the heat seal layer would also contain polyethylene. If the container includes polypropylene, then the heat seal layer would also contain polypropylene. Other similar materials combinations are also possible.

Support layer 102 may be optional in the laminate 114. If included, it may be polyethylene terephthalate (PET), nylon, or other structural polymer layer and may be, in some approaches, about 0.5 to about 1 mil thick.

Next, the membrane layer **104** may be one or more layers configured to provide induction heating and/or barrier characteristics to the seal **10**. A layer configured to provide induction heating is any layer capable of generating heat upon being exposed to an induction current where eddy currents in the layer generate heat. By one approach, the membrane layer may be a metal layer, such as, aluminum foil, tin, and the like. In other approaches, the membrane layer may be a polymer layer in combination with an induction heating layer. The membrane layer may also be or include an atmospheric barrier layer capable of retarding the migration of gases and moisture at least from outside to inside a sealed container and, in some cases, also provide induction heating at the same time. Thus, the membrane layer may be one or more layers configured to provide such functionalities. By one approach, the membrane layer is about 0.3 to about 2 mils of a metal foil, such as aluminum foil, which is capable of providing induction heating and to function as an atmospheric barrier.

Layer **106** may be an insulation layer or a heat-redistribution layer. In one form, layer **106** may be a foamed polymer layer. Suitable foamed polymers include foamed polyolefin, foamed polypropylene, foamed polyethylene, and polyester foams. In some forms, these foams generally have an internal rupture strength of about 2000 to about 3500 g/in. In some approaches, the foamed polymer layer **106** may also have a density less than 0.6 g/cc and, in some cases, about 0.4 to less than about 0.6 g/cc. In other approaches, the density may be from about 0.4 g/cc to about 0.9 g/cc. The foamed polymer layer may be about 1 to about 5 mils thick.

In other approaches, the layer **106** may be a non-foam heat distributing or heat re-distributing layer. In such approach, the non-foam heat distributing film layer is a blend of polyolefin materials, such as a blend of one or more high density polyolefin components combined with one or more lower density polyolefin components. Suitable polymers include but are not limited to, polyethylene, polypropylene, ethylene-propylene copolymers, blends thereof as well as copolymers or blends with higher alpha-olefins. By one approach, the non-foam heat distributing polyolefin film layer is a blend of about 50 to about 70 percent of one or more high density polyolefin materials with the remainder being one or more lower density polyolefin materials. The blend is selected to achieve effective densities to provide both heat sealing to the container as well as separation of the liner from the seal in one piece.

When used in the seal **10**, effective densities of the non-foam heat distributing polyolefin layer **106** may be between about 0.96 g/cc to about 0.99 g/cc. Above or below this density range, unacceptable results are obtained with non-foam layers because the layer provides too much insulation or does not effectively distribute heat. By another approach, the non-foam heat distributing layer is a blend of about 50 to about 70 percent high density polyethylene combined with low to medium density polyethylene effective to achieve the density ranges described above.

In addition, effective thicknesses of the non-foam heat distributing layer are selected to achieve such performance in combination with the density. One approach of an effective thickness may be about 2 to about 10 mils. In other approaches, layer **106** may be about 2 to about 5 mils thick, in other approaches, about 2 to about 4 mils thick, and in yet other approaches, about 2 to about 3 mils thick. Thicknesses outside this range tend to be unacceptable for heat redistribution because the layer does not provide enough insulation or does not effectively distribute heat as needed to achieve the dual performance characteristics of liner separation and seal member bonding.

On top of the lower laminate **14** is an optional, outer polymer support layer **108**, which may be a non-foam PET, nylon, or other structural-type polymer layer(s) such as polyolefin or copolymers thereof. In one approach, outer layer **108** may be the one or more non-foam, polymer film or layers (or the non-foam, polymer sub tab layers discussed herein) mentioned above to provide concentric stability to the sealing member and polymer foam layer underneath it. In one form, layer **108** may be an asymmetrical polyester film having an upper layer of an amorphous polyester and a lower layer of a crystallized polyester layer. The amorphous polyester layer may have a lower melting point than the crystallized polyester and may aid in achieving a good bond with the upper laminate **12** and improve processing over hot rollers and other equipment during seal manufacture. In one approach, the layer **108** is a co-extruded layer with the crystallized layer being thicker than the amorphous layer. In the seal, the amorphous layer may form the bond with the upper laminate **12** and form the upper surface **32** of the lower laminate **14**. The upper laminate **14** may also include other layers as needed for a particular application, which may be layers in between the various layers discussed herein as appropriate for a particular application. In other approaches, layer **108** may be one or more layers of a polyolefin. In some approaches, to provide concentric stability, layer **108** may be about 1 to about 5 mils thick and have a density of about 0.9 to about 1.5 g/ml (in some cases about 0.9 to about 1.2, and in other cases, about 0.9 to about 1.0 g/ml, and in yet other cases about 0.9 to about 0.96 g/ml).

Turning to FIG. 4 for a moment, each of the layers of FIG. **3** may also be bonded to the layer adjacent to it via an optional adhesive or tie layer **110**. These adhesive or tie layers may be the same, as shown in the exemplary seal of FIG. **4**, but may also be different in composition. The adhesives useful for any of the optional adhesive or tie layers described herein include, for example, ethylene vinyl acetate (EVA), polyolefins, 2-component polyurethane, ethylene acrylic acid copolymers, curable two part urethane adhesives, epoxy adhesives, ethylene methacrylate copolymers and the like bonding materials. Other suitable materials may include low density polyethylene, ethylene-acrylic acid copolymers and ethylene methacrylate copolymers. By one approach, any optional adhesive layers may be a coated polyolefin adhesive layer. If needed, such adhesive layers may be a coating of about 0.2 to about 0.5 mil (or less) adhesive, such coated ethylene vinyl acetate (EVA), polyolefins, 2-component polyurethane, ethylene acrylic acid copolymers, curable two part urethane adhesives, epoxy adhesives, ethylene methacrylate copolymers and the like bonding materials.

As explained previously, the layers forming the upper laminate may extend only partially across the sealing members **10** as generally shown in FIGS. **3** and **4**. In alternative approaches, the layers **122** and **120** may also extend the full width and full surface area of the sealing members as generally shown in FIGS. **10** and **11**. Layers **122** and **120** will be explained further below in the context of FIG. **3**, but it will be appreciated that full layers of these portions will have similar characteristics and constructions.

Turning back to FIG. **3**, one approach of the circular segment portion forming the upper laminate **12** will be described further. In this approach, the laminate **12** includes a layer of heat activated adhesive or a heat activated bonding layer **120** and a corresponding or overlapping upper polymer support layer **122** where the adhesive layer **120** partially bonds **126** the support layer **122** to the upper surface **32** of the lower laminate **14** to form both the tab portion **16** and the bonded portion **30**. The upper polymer support layer **122** may be PET,

## 11

nylon, or other structural-type polymer layer(s). As noted above, layer 120 and layer 122 may also extend the full width and surface area of the seal 10.

In the approach of FIG. 3, the upper laminate also includes a partial layer 124, which is shorter or smaller than layers 120 and 122 of the laminate 112, and called a tab stock. The tab stock 124 is adhered or bonded to the adhesive layer 120 on a top surface thereof, but is not bonded to the lower laminate 14 (or any sub-tab polymer layer) in the final assembly. However, in optional approaches, the tab 16 may also be formed without a tab stock 124 and, instead, utilize a part layer of adhesive corresponding only to the bond area 30. (This optional way of forming the tab 16 may be utilized on any of the seal approaches described herein.)

When using the tab stock 124, the tab 16 is defined or formed via the tab stock 124 that extends only part way across the upper laminate 12. More specifically, the tab stock 124 forms the tab 16 because it bonds to the heat-activated bonding layer 120 and generally prevents layer 122 (and any layers above) from adhering to the upper surface 32 of the lower seal laminate 14 (or sub-tab polymer layer) across at least a portion thereof as generally shown in FIGS. 3 and 4. That is, a top surface of the tab stock 124 is adhered to a lower portion of the heat-activated bonding layer 120. A bottom surface of tab stock 124 is adjacent to, but not bonded to, the upper surface 32 of the lower laminate 14 (or sub-tab polymer layer) to form the tab 16. In one aspect, the tab stock 124 is formed of polyester, such as polyethylene terephthalate (PET), or paper. By one optional approach, a lower surface of the tab stock 124 may be coated with a release material, for example silicone. The optional release coating minimizes the possibility that the tab stock 124 will become adhered to the upper surface 32 of the lower laminate 14 during the heat sealing or induction heat sealing process. However, such release coatings are not typically necessary. As generally shown in at least FIGS. 3 and 4, the tab stock 124 permits the tab structure 16 to pivot or hinge upwardly along a boundary line 34 to form the tab 16. By this approach, the tab stock 124 and formed tab 16 are defined wholly within a circumference or perimeter 22 of the seal.

The heat-activated bonding layer 120 may include any polymer materials that are heat activated or heated to achieve its bonding characteristics or application to the seal. By one approach, the heat-activated bonding layer may have a density of about 0.9 to about 1.0 g/cc and a peak melting point of about 145° F. to about 155° F. A melt index of the bonding layer 120 may be about 20 to about 30 g/10 min (ASTM D1238). Suitable examples include ethylene vinyl acetate (EVA), polyolefin, 2-component polyurethane, ethylene acrylic acid copolymers, curable two-part urethane adhesives, epoxy adhesives, ethylene methacrylate copolymers and the like bonding materials. As shown, the heat activated bonding layer 120 extends the full width of the laminate segment 12 (but not the full width or length of the entire seal 10 or the entire lower laminate 14). In other approaches, the laminate 12 may only include a partial layer of adhesive and, thus, not use the tab stock layer 124 discussed above. In other approaches, the bonding layer 120 extends the full width of the seal and is partially bonded to the lower laminate portion and partially bonded to the tab stock 124. In yet other approaches, the bonding layer 120 is partially bonded to the polymer support layer 108.

By one approach, the heat-activated bonding layer 120 is EVA with a vinyl acetate content of about 20 to about 28 percent with the remaining monomer being ethylene in order to achieve the bond strengths to securely hold the upper laminate to the lower laminate. In some cases, a vinyl acetate

## 12

content lower than 20 percent is insufficient to form the robust structures described herein. By one approach, bonding layer 120 may be about 0.5 to about 3.5 mil of EVA, in other approaches about 0.5 to about 2.5 mils of EVA, in other approaches, about 0.5 to about 1.5 mils of EVA and, in yet other approaches, about 0.5 to about 1.0 mils of EVA; however, the thickness can vary as needed for a particular application to achieve the desired bonds and internal strength.

With sealing members including a tab defined wholly within a perimeter of the sealing member, upon pulling of the tab, there is a generally stress focal point right at the juncture or hinge joint 34 where the tab pivots upwardly. Generally, the stress upon tab pulling radiates downwardly and away from this hinge joint into the layers below the tab and, in some cases, results in a tearing of the layer immediately below the tab. This failure tends to occur more often in prior tabbed sealing members when the layer immediately below the tab is a foamed polymer. In the present approaches, the structural support layer 108 is also advantageous because it provides a more rigid, non-foam layer underneath the focal point of the tab pulling stress to provide a more robust laminate structure upon tab pulling. In the present approaches, the pulling stresses are dissipated throughout a denser, more rigid layer providing a more robust tab capable of withstanding even stronger heat seal bonds to containers. The density of the non-foam polymer layer under the tab, in some approaches, may be about 0.9 to about 1.2 g/cc. The sub-tab layer may also be about 1 to about 5 mils thick.

FIGS. 5 and 6 show yet another alternative approach of a sealing member 101 described herein. In this approach, a lower laminate 114 includes just a lower sealant or heat seal layer 100 combined with a membrane layer 104 bonded together with an optional adhesive layer 110. The upper laminate 12 or segment may also include similar layers as the version discussed above. To this end, the segment 12 may include an upper polymer support 122, a heat activated bonding layer 120, and the tab stock 124. The composition of these layers is similar to the version discussion above and will not be discussed further. In this approach, the lower laminate may be from about 1 to about 5 mils thick, and in other approaches, about 1 to about 3 mils thick.

The approach of FIGS. 5 and 6 is advantageous because it presents an exposed membrane layer (often a foil layer) as a portion of, and in some cases, the majority of the top surface of the sealing member 101. Additionally, in view of the relatively thin laminate 114, the sealing member 101 can be opened by either a consumer pulling on the tab 16 to peel the sealing member from the container rim or, alternatively, exposed portions 200 of the seal (that is, the portions of the seal not covered by the upper laminate segment 12) can easily be punched through or pierced by a consumer. This enables push/pull functionality to the seal—that is, push or pierce through the lower laminate 14 and pulling of the tab 16 to peel the seal 10 from the container. FIG. 7 shows an approach with the tab stock 124 formed from a PET layer while FIG. 8 shows an alternative approach with the tab stock 124 formed from a paper layer; however, the tab stocks of these figures may also be interchangeable.

FIG. 7 illustrates the seal of FIG. 5 or 6 in an exemplary two-piece seal and liner assembly 300. The other seals described herein may also be used in a similar arrangement. In this approach, a top surface of the sealing member 101 is temporarily bonded to a liner 302 shown as an optional pulp backing in FIG. 7. The liner 302 is temporarily adhered to seal 101 via an intermediate layer 304, which in this approach, is a heat-activated layer of wax or microcrystalline wax. Prior to heat sealing (by induction, conduction, or the like) to a con-

tainer rim, the wax layer 304 bonds the liner 302 to the seal 101. As part of the heating process to bond the seal 101 to a container, heat (in some approaches, induction heating from the metal layer) flows upwardly in the seal and activates or melts the wax 304 to release the bond between the liner 302 and the sealing member 101, which separates the two components. In some approaches, the wax is melted and absorbed by the liner 302. Other releasable layers that provide a temporary bond between layer 104 and 302 may also be used.

As can be appreciated, for this separation to occur cleanly and properly, the wax needs to melt across the entire surface area of the seal 101. With prior seals having a full layer of film and in some cases a full layer of adhesive, there was additional material at the center portion of the seal that the upwardly directed heat needed to transfer through. As the center portions of the seal are farthest from the induction coils and, thus, generating the lowest levels of induction heat, the center of the seal was previously prone to not generating sufficient heating in a two-component assembly when an upper laminate included full layers forming the tab. This poor central upwards heat transfer was often made worse if the seal had an insulation layer that further limited upward heat transfer, or if the seal was large (such as about 60 mm or greater).

The seal of FIG. 7, for example, eliminates the additional tab forming layers at the center and central portions of the seal 101 so that these areas with the weakest eddy currents in induction sealing do not need to generate high levels of heat to flow through additional layers of material in order to reach and melt the center wax areas. Thus, the seal of FIG. 7 provides an improved two-piece seal and liner assembly even with a tab defined wholly within a perimeter or circumference of the seal. Moreover, because the center of the seal is exposed, the upper laminate 12 can be thicker than normally used in tabbed seals and, in some approaches, be greater than about 5 mils, and in other approaches be about 5 to about 10 mils thick. This layer can also include other structural support layers without the problem of hindering upwardly directed heat flow. To this end, laminate 12 may include thick polymer and/or thick foam layers to improve tab rigidity.

In some approaches, the liner 302 can be formed of one or more layers of cardboard, pulp board, or a synthetic compressing agent (such as a synthetic foam or synthetic fibers) that is effective for absorbing the release layer 304, such as wax, upon being activated by heating. In one approach, the liner 302 may include a layer of foamed plastic material to which a paper layer (not shown) has been adhered to a bottom surface thereof. In this approach, the paper layer is the layer in contact with the release layer 304 for absorbing the molten wax or other activated components thereof. By another approach, the liner 302 may have a thickness in the range from about 400 to about 1800 microns. Synthetic foam or fibers may also be useful as materials for the liner if they are formed into a layer with a suitable compression factor comparable to pulp board of the type traditionally used in induction seals. For example, low density polyethylene (LDPE), coextruded LDPE, polypropylene (PP), and polystyrene (PS) foam or fibers may also be used as the liner. The synthetic material selected should have a sufficient absorbency, suitable pore volume, and structure to absorb substantially all of the wax used in the seal. The dimensions of the compressing agent absorbing material will vary according to the application and the size of the opening of the container and size and construction of the closure being used.

By one approach, the release layer 304 may be a wax layer. The wax may include any suitable wax material which will melt within the temperature range to which the sealing member is to be subjected by an energy source during the induction

sealing process. For example, the wax layer may include paraffin, microcrystalline waxes, and blends thereof. By one approach, the wax layer may comprise a blend of paraffin wax and microcrystalline wax wherein the proportion of microcrystalline wax used in the wax layer is adjusted to provide the wax layer being formulated to enhance the ability of the wax to be absorbed by the liner. Alternatively, the wax layer may include microcrystalline wax modified with other polymeric additives to enhance its initial bonding properties. For instance, the wax layer may comprise microcrystalline wax modified with at least one of ethylene vinyl acetate and polyisobutylene.

In general, the application of induction energy to the sealing member heats the membrane layer 104 to a temperature, in some approaches, from about 300 to about 450° F. The volume or thickness of the wax layer, therefore, should be selected such that substantially all of the wax will melt during the manufacturing process and be absorbed by the compressing agent.

FIGS. 8 and 9 schematically show some of the relative features of the seal when viewed from above and the unique characteristics of the circular segment upper laminate 12. As shown in FIG. 10, the total upper laminate segment portion 12 may be defined by an angle  $\alpha 1$  between radius lines extending from the center C to the chord endpoints 24 and 26 of about 125° to about 150°, in other approaches, about 130 to about 140°, and in yet other approaches, about 130 to about 138°. This forms an upper laminate segment portion 12 that covers about 10 to about 40 percent of the upper surface of the seal, in other approaches about 14 to about 35 percent of the seal, in yet other approaches, about 20 to about 30 percent of the seal. In this manner, the upper surface of the seals herein are formed from a minor portion of the top layer from the upper laminate portion 12 and by a major portion from the top layer of the lower seal laminate 14.

The tab 16 of the upper laminate circular segment may also define a second circular segment and may be defined by a second angle  $\alpha 2$  between radius lines extending outwardly from the center C to secondary chord endpoints 300 and 302 on opposite sides of a chord defining the pivot line 34 of about 90 to about 120°, in other approaches, about 100 to about 115°, and in yet other approaches, about 105 to about 112°. In this manner, the seals define a tab 16 that wholly defined within a perimeter of the seal in a ratio of tab surface area to the surface area of the bond area 30 of about 1:1 to about 3:1 and in some approaches, about 1:1 to about 2:1. These ratios are achieved even when the upper laminate portion 12 is less than about 50 percent of the seal, in some approaches, less than about 40 percent of the seal, and in yet other approaches, less than about 35 percent of the seal's upper surface area.

Turning to FIG. 9, another schematic of an exemplary sealing member is shown showing various relative relationships between the upper laminate circular segment portion 12 and the upper surface 32 of the lower laminate 14 effective for the sealing member to function as an overlapping tab on several different configurations of lower laminate. In one approach, the upper laminate circular segment 12 has a total height H that is about 15 to about 40 percent (in some approaches, about 20 to about 30 percent) of the total length 60 of the sealing member with the total length of the exposed lower laminate portion 32 being about 60 to about 85 percent (in other approaches, about 70 to about 80 percent) of the total sealing member length. Thus, in some approaches a ratio of the circular segment height to the length of the exposed lower laminate 32 may be about 0.2 to about 0.7.

Turning to FIG. 10, one example of a sealing member 200 including a sub tab layer 202 is shown. In this approach, many

## 15

of the layers are similar in position and composition to those already discussed above, and these layers will not be discussed further in this alternative approach. In this approach, the sub tab layer 202 is bonded to the lower laminate 214 and, in particular, to the upper surface 32 and in the approach of FIG. 10, the foil layer 104 of the lower laminate 214. In other approaches, sub tab layer 202 may be bonded to a foam layer above the foil layer 104. The sub tab 202 is not bonded to the tab 16 or the upper laminate 212. While the sub tab layer 202 is shown bonded to a particular lower laminate, the structure of the lower laminate is not particular limited and can be any single or multi-layer film structure, such as the other lower laminates discussed herein.

The sub tab 202 may be a paper layer adhered to the lower laminate via a hot melt adhesive or a film layer (polyolefin, polyester, nylon, etc.) heat bonded or adhered to the lower laminate via a thin coating of adhesive. In some approaches, the sub tab 202 may be about 1 to about 5 mils thick and, in other approaches, about 1 to about 2 mils thick. The sub tab layer may be coextensive with the tab stock 124, which may also be a paper layer so that this approach presents a paper to paper interface between the tab 16 of the upper laminate 12 and the lower laminate 214. While the sub tab is shown in the figures to be a partial layer, the sub tab layer may also extend the entire width and surface area of the seal (not shown) as needed for a particular application as discussed previously and as discussed more below. The sub tab layer 202 provides structural support and aids in minimizing the formation of folds, creases, wrinkles and other deformities when the tab layer is applied to the lower laminate. The sub tab layer 202 may be particularly advantageous in providing structural support for lower laminates that are 3 mils or less as these are the most prone to such structural defects during handling and cap sealing and, in some cases, when combined with a gripping tab. For example, the sub tab layer 202 may aid in providing the concentric structural stability discussed previously during a cap heat sealing process.

In FIG. 10, the sealing member 200 may also include optional upper layers 220 above the tabbed seal. In one approach, the upper layers may provide additional structural support and may include a paper or cellulose backing layer 222 and an adhesive layer 224. The paper backing layer 222 may be about 5 to about 10 mils of paper backing. Adhesive layer 224 may be any of the exemplary adhesive layers discussed above. This approach provides a robust tab 16 but still provides easy access to the container contents by, for instance, piercing or punching through the foil layer via the portions of the seal 200 not covered by the upper laminate 12.

FIG. 11 provides yet another example of a sealing member 300 utilizing the sub tab layer 202 combined with a lower laminate 214, which in this approach is similar to that described above with FIG. 10. It will be appreciated, however, that the lower laminate 214 may be any single or multi-layer laminate as needed for a particular application, such as any of the lower laminates discussed previously.

In this approach, a tab 215 is formed from a polymer layer 350, which may be a structural polymer layer such as polyester (PET), PEN, nylon, or the like. Above the layer 350 may be an additional support layer, such as backing layer 222 (which may be bonded to layer 350 via adhesive layer 224, which is not shown in FIG. 11). In this approach, the tab is formed via a partial bond or adhesive layer, which does not extend the full length of the seal 300, of a composite adhesive film or laminate 352 formed from a polyester core layer 354 sandwiched between two outer layers of a heat bondable

## 16

materials 356 and 358. Composite film layer 352 may be about 2 to about 8 mils thick, and in some approaches, about 3 to about 4 mils thick.

The heat bondable materials 356 and 358 may include any polymer materials that are heat activated or heat applied to achieve its bonding characteristics. By one approach, the heat-bondable layer may have a density of about 0.9 to about 1.0 g/cc and a peak melting point of about 145° F. to about 155° F. A melt index of the heat bondable material may be about 20 to about 30 g/10 min (ASTM D1238). Suitable examples include ethylene vinyl acetate (EVA), polyolefin, 2-component polyurethane, ethylene acrylic acid copolymers, curable two-part urethane adhesives, epoxy adhesives, ethylene methacrylate copolymers and the like bonding materials.

By another approach, the heat bondable material is EVA with a vinyl acetate content of about 20 to about 28 percent with the remaining monomer being ethylene in order to achieve the bond strengths in order to securely hold the upper laminate to the lower laminate. A vinyl acetate content lower than 20 percent is insufficient to form the robust structures described herein. By one approach, layer 352 may include upper and lower layer 356 and 358 about 0.5 to about 1.5 mil of EVA and, in other approaches, about 0.5 to about 1.0 mils of EVA; however, the thickness can vary as needed for a particular application to achieve the desired bonds and internal strength.

Sealing member 300 may also include the sub tab layer 202 discussed above to provide structural support to the layers above and below the tab. The sub tab layer 202, in this approach, may have similar characteristics as the sub tab layer discussed above. The layer 202 is bonded to the upper surface of the lower laminate and not bonded to the layer(s) 350 forming the tab 215.

In alternative approaches, the sub tab layer 202 may, instead of being coextensive with the primary tab 16 or any tab stock 124 thereof, may extend laterally beyond the boundaries of the tab 16 or tab stock 124. In some approaches, the sub tab layer could be coextensive with the upper laminate or extend over half of the sealing member. In this approach, the sub tab layer could help improve adhesion of the upper laminate to the lower laminate. For instance, if a foam layer is used for the sub tab 202, then the sub tab could extend beyond the tab and tab stock further towards the center of the seal C to engage the bonding area 128, for example, to improve the bond therewith. In this approach, a strong bond would be needed between the extended sub tab layer 202 and the upper surface of the lower laminate (such as the foil layer).

In another approach, if the sub tab layer 202 was a paper or other absorbent material, then temporarily bonding-type materials or adhesives could be applied to the upper surface of the sub tab to temporarily bond the upper surface of the sub tab to the tab 16 or the tab stock 124 in the upper laminate. In this manner, the temporary bond between the sub tab layer 202 and layers above it in the upper laminate would temporarily bond and/or hold the tab to the lower laminate in order to secure the upper tab substrate for maintaining concentric and/or lateral stability of the entire liner layers, including the tab interface to the lower layer, prior to heat activation and during normal handling and cap assembly.

By one approach, the temporary bond between the sub tab and upper laminate tab or tab stock could be by a wax layer, such as the previously described waxes. In this manner, upon heating to secure the sealing member to the container rim, the heat generated would melt the wax, which would release the tab or tab stock from the sub tab layer and free the tab for normal use. The wax could then be absorbed into the paper or

other absorbent material of the sub tab layer similar to how wax is melted and absorbed by a liner in the two-piece assembly constructions described above. The wax could be applied or coated to the top surface of the sub tab layer prior to construction of the sealing member or applied in-line to this component during seal assembly. Alternatively, the temporary bond between the sub tab layer and the upper layers above it could employ alternative release mechanisms, such as dissimilar polymers (such as for example, different polymers on the sub tab and adjacent layers), slip additive loadings to the sub tab or other adjacent layers, cold seal release technology that may provide a temporary bond but would be easily peelable for a consumer to pivot the tab upwardly. In addition, the sub tab layer may further be formed of synthetic short non-woven fibers that are intertwined to form an absorbent sheet, similar to that described in U.S. Pat. No. 7,850,033, which is incorporated herein by reference in its entirety. When forming a temporary bond with the sub tab layer 202, and in some approaches due to the location in the laminate structure, any wax that may be used to form the temporary bond may be a wax with a higher melt point than the waxes discussed above with the two-piece seal and liner constructions. This higher melt point wax can be used in this location without impeding any functionality of the seal and release of the sub tab layer from the other layers during heat sealing. This is because the sub tab layer is positioned closer to the induction heating layer in some approaches.

In summary, the disclosure herein provide for, among other features, a tabbed sealing member for sealing to a rim of a container where the tabbed sealing member includes an overlapping upper laminate that may include a lower seal portion having a top surface with a total surface area and including a heat sealable layer configured for heat sealing to a container rim, an upper laminate at least partially bonded to the top surface of the lower seal portion to form a gripping tab defined wholly within a perimeter of the lower seal portion. In some approaches, the upper laminate has a top surface with a surface area less than the total surface area of the lower seal portion top surface and forming a circular segment defined by an edge forming a chord extending across the lower seal portion and spaced from a center of the tabbed sealing member. In some approaches, the sealing member further includes a sub tab layer coextensive with at least the gripping tab or extending the full extent of the seal. The sub tab layer is bonded to the top surface of the lower seal portion and not bonded to the gripping tab. The sub tab layer may be paper, polymers, polyester, and the like materials. In some approaches, a full backing layer is adhered to both the top surface of the upper laminate and the top surface of the lower seal portion. In some approaches, the backing layer is paper about 5 to about 10 mils thick.

In optional approaches, the tabbed sealing member may also include wherein an upper laminate with a heat activated bonding layer forming the at least partial bond to the top surface of the lower seal portion or a tab stock bonded to the heat activated bonding layer but not bonded to the top surface of the lower seal portion to form the gripping tab. In other approaches, an upper surface of the tabbed sealing member may be partially defined by a minor portion of the top surface of the upper laminate and a major portion of the top surface of the lower seal portion. The upper surface of the tabbed sealing member may also be temporarily bonded to a liner with portions of the liner are temporarily bonded to the top surface of the upper laminate and other portions of the liner are temporarily bonded to the top surface of the lower seal portion.

In some approaches, the lower seal portion may have a thickness and composition configured to be pierced through portions of the tabbed sealing member not covered by the upper laminate.

5 In some approaches, the circular segment forming the upper laminate may be defined by a sweep angle of the formula  $2 \text{ arc cos}(H1/\text{radius})$ . In some approaches, this angle may be about 125 to about 150°. In other approaches, the tab of the upper laminate is a circular segment being less than a 10 semicircle and defined by a second sweep angle of the formula  $2 \text{ arc cos}(H2/\text{radius})$ . In some approaches, this angle may be about 90 to about 120°.

The circular segment of the upper laminate, in some forms, may cover about 10 to about 40 percent of the upper surface 15 of the tabbed sealing member with the remainder of the upper surface being the top surface of the lower seal portion.

The lower seal portion, in some alternative approaches, may include a variety of different materials and layers. For instance, the lower seal portion may include a metal foil, and 20 the top surface of the lower seal portion may be the metal foil. The lower seal portion may also include a foamed polymer, or the top surface of the lower seal portion may be a polymer film selected from polyolefin materials and polyester materials.

In other approaches, a tabbed sealing member for sealing to 25 a rim of a container is described that includes a lower seal portion having a top surface with a total surface area and including a heat sealable layer configured for heat sealing to a container rim. The seal further includes an upper laminate at least partially bonded to the top surface of the lower seal 30 portion to form a gripping tab defined wholly within a perimeter of the lower seal portion. The partial bond is formed by a composite layer of a polyester sandwiched between heat bondable materials on opposite sides of the polyester. The seal also includes a sub tab layer coextensive with the gripping tab. The sub tab layer is bonded to the top surface of the 35 lower seal portion, but not bonded to the gripping tab. In some alternative approaches, the tabbed sealing member includes a layer of polyester and a paper backing layer.

In optional approaches, the tabbed sealing members herein 40 may include multi-component segmentation with a separate layer segmented from and adjacent to the upper laminate forming the tab. That is, the upper laminate may be adjacent to and separate from another segmented layer also bonded to the lower seal portion but distinct from the upper laminates 45 discussed above. The segmented layer may be a single or multi-layer laminate that is the same thickness as the upper laminate forming the tab in the various approaches above. The segmented layer may be a paper layer.

It will be understood that various changes in the details, 50 materials, and arrangements of the process, liner, seal, and combinations thereof, which have been herein described and illustrated in order to explain the nature of the products and methods may be made by those skilled in the art within the principle and scope of the embodied product as expressed in 55 the appended claims. For example, the seals may include other layers within the laminate and between the various layers shown and described as needed for a particular application. Adhesive layers not shown in the Figures may also be used, if needed, to secure various layers together. Unless 60 otherwise stated herein, all parts and percentages are by weight.

What is claimed is:

1. A container and cap assembly including a concentrically 65 stable tabbed sealing member with foam for sealing to a rim surrounding an opening of the container, the assembly comprising:

a container with a rim surrounding an opening thereof;

19

a cap for closing the opening of the container; a multi-layer laminate forming the concentrically stable tabbed sealing member and including an upper laminate portion with one or more layers and partially bonded to a lower laminate portion; a tab stock polymer layer extending partway across the sealing member, the tab stock polymer layer bonded to one of the layers in the upper laminate portion and not bonded to the lower laminate portion, the tab stock polymer layer and the portion of the upper laminate bonded to the tab stock polymer layer form a gripping tab defined wholly within a perimeter of the sealing member, the multi-layer laminate bonded to the container rim; the lower laminate portion below the gripping tab including at least a seal layer for bonding to the container rim, a metal layer for heating the seal layer, and a polymer foam layer above the metal layer; a polymer film sub-tab layer between the polymer foam layer and the gripping tab; and the polymer film sub-tab layer coextensive with at least the gripping tab at its periphery thereof to provide structural support to the polymer foam layer at its periphery, thereby, protecting the structural integrity of the polymer foam layer from effects of heat sealing the tabbed sealing member to the container rim.

2. The assembly of claim 1, wherein the polymer film sub-tab layer is bonded to the polymer foam layer and not bonded to the gripping tab.

3. The assembly of claim 2, wherein the polymer film sub-tab layer is directly bonded to the polymer foam layer.

4. The assembly of claim 1, wherein the polymer film sub-tab layer is bonded to the polymer foam layer and not bonded to the tab stock polymer layer.

5. The assembly of claim 1, wherein the polymer film sub-tab layer is a polyolefin.

6. The assembly of claim 1, wherein the polymer film sub-tab layer is about 1 to about 5 mils thick.

7. The assembly of claim 1, wherein the polymer foam layer has an internal rupture strength of about 2000 to about 3500 grams per inch.

8. The assembly of claim 1, wherein the polymer foam layer has a density of about 0.4 to about 0.6 grams per cubic centimeter.

9. The assembly of claim 1, wherein the partial bond between the upper laminate portion and the lower laminate portion is through the polymer film sub-tab layer.

10. The assembly of claim 1, wherein the upper laminate portion includes a heat-activated bonding layer that is partially bonded to the polymer film sub-tab layer and partially bonded to the tab stock polymer layer.

11. The assembly of claim 10, wherein the heat-activated bonding layer is selected from the group consisting of ethylene acrylic acid copolymers, curable two-part urethane adhesives, epoxy adhesives, ethylene methacrylate copolymers and mixtures thereof.

12. The assembly of claim 10, wherein the upper laminate portion includes a top polyester layer above the heat-activated bonding layer.

13. The assembly of claim 1, wherein, after heat sealing, the polymer foam layer has concentric stability where the structural integrity of the polymer foam layer remains substantially consistent at its periphery relative to a portion of the polymer foam layer radially inward from the periphery.

20

14. The assembly of claim 1, wherein an inner surface of the cap includes a downwardly extending bead substantially aligned with the container rim.

15. A laminate for forming a concentrically stable tabbed induction sealing member with a foam layer for sealing to a rim surrounding a container opening, the laminate comprising:

a multi-layer laminate including an upper laminate portion with one or more layers and partially bonded to a lower laminate portion to form a gripping tab when the laminate is formed into the concentrically stable tabbed sealing member;

the lower laminate portion including at least a heat seal layer for bonding to the container rim after the laminate is formed into the concentrically stable tabbed sealing member, a metal layer for heating the heat seal layer, and a polymer foam layer above the metal layer;

a non-foam polymer sub-tab layer positioned between the polymer foam layer and the upper laminate;

a tab stock polymer layer extending partway across the laminate, the tab stock polymer layer bonded to one of the layers in the upper laminate portion and not bonded to the lower laminate portion; and

when the laminate is formed into the concentrically stable tabbed induction sealing member and induction bonded to the container rim, the non-foam polymer sub-tab layer is arranged and configured to provide structural support to the polymer foam layer at its periphery, thereby, protecting the structural integrity of the polymer foam layer from effects of induction heat sealing the formed concentrically stable tabbed sealing member to a container rim.

16. The laminate of claim 15, wherein the non-foam polymer sub-tab layer is bonded to the polymer foam layer and partially bonded to the upper laminate portion.

17. The laminate of claim 15, wherein the non-foam polymer sub-tab layer is bonded to the polymer foam layer and not bonded to the tab stock polymer layer.

18. The laminate of claim 15, wherein the partial bond between the upper laminate portion and the lower laminate portion is through at least the non-foam polymer sub-tab layer.

19. The laminate of claim 15, wherein, after the laminate is formed into the concentrically stable tabbed sealing member and after heat sealing to a container rim, the polymer foam layer has concentric stability where the structural integrity of the polymer foam layer remains substantially consistent at its periphery relative to a portion of the polymer foam layer radially inward from the periphery.

20. The laminate of claim 15 formed into the concentrically stable tabbed sealing member.

21. The laminate of claim 20, wherein the formed concentrically stable tabbed sealing member is combined with a cap having an inner surface with a downwardly extending bead substantially aligned with the container rim.

22. The laminate of claim 15, wherein the polymer foam layer has an internal rupture strength of about 2000 to about 3500 grams per inch.

23. The laminate of claim 22, wherein the polymer foam layer has a density of about 0.4 to about 0.6 grams per cubic centimeter.

24. The laminate of claim 15, wherein the upper laminate portion includes a heat-activated bonding layer that is partially bonded to the non-foam polymer sub-tab layer and partially bonded to the tab stock polymer layer.

\* \* \* \* \*